

## UNITED STATES PATENT OFFICE

2,280,709

PROCESS FOR THE MANUFACTURE OF  
MEERSCHAUM PIPES

Ernest Lichthau, New York, N. Y.

No Drawing. Application October 12, 1939,  
Serial No. 299,158

4 Claims. (Cl. 18—55)

This invention relates to a method for the manufacture of pipes and cigarette holders of meerschaum and similar meerschaum articles. It relates in particular to the manufacture of articles of the named type where a low grade meerschaum, meerschaum compositions, meerschaum waste or meerschaum powder is used as a starting material.

As generally known, two main requirements dominate the manufacture of this type articles.

The finished product must be sufficiently resistant to mechanical stresses and to breakage and it must have the aspect, the color and the lustre of a pipe which is made from a first grade meerschaum material.

Numerous methods have been suggested to comply with these requirements.

In order to obtain the lustre and the soft tint as well as the color of a superior meerschaum pipe a treatment with wax has been considered indispensable.

For this purpose the shaped article has been impregnated with wax or immersed in wax or in mixtures of wax with certain oils or oleaginous materials.

The thus treated article is fragile and has no resistance to impacts or shocks. It has also the tendency to crack in use.

In order to remedy this insufficiency the shaped and waxed article is treated or impregnated with varnishes or lacquers and is subsequently hardened by a heat treatment.

The results of these known treating methods of meerschaum articles however have not been satisfactory in as much as the mechanical resistance and the lustre of the finished products is greatly inferior to a pipe which is cut from a first quality meerschaum.

Besides, the known treating methods which include a plurality of working steps are rather complicated. Furthermore it often happens that seemingly by the interaction of the wax and the coating lacquers blisters are created when the pipe is heated which blisters create an exfoliation of the coatings.

The above mentioned drawbacks of the known methods of manufacturing meerschaum pipes and similar articles are obviated by this invention.

The latter is based on the surprising discovery that all the requirements of a highest grade meerschaum pipe may be satisfactorily fulfilled without subjecting the pipes to the customary tiresome wax treatment. In accordance therewith it may be specifically pointed out that the

invention is confined to meerschaum smoker articles for which a waxed treatment has been hitherto considered essential; therefore the elimination of this treating step signifies an invention. However, the invention has no bearing on the application of materials like briar wood which is largely used for the manufacture of tobacco pipes, which are coated for instance with solutions of a mixture of urea resin and nitrocellulose.

10 It is therefore an object of the invention to produce a meerschaum pipe or similar meerschaum article particularly from a low quality meerschaum and from meerschaum compositions or powders without subjecting the article to a waxing treatment and nevertheless to obtain by the sole application of synthetic resin solutions an article which equals in outer appearance, lustre, color and tint to the genuine high grade article.

15 It is another object of the invention to increase the mechanical resistance of the pipe to such an extent that it not alone equals but is superior to a pipe which is made from the highest grade meerschaum.

20 It is a further object of the invention to prevent the creation of blisters when the pipe is heated which cause exfoliation of the coatings and render the pipe practically useless.

25 Other objects of the invention will become apparent when the description proceeds.

30 As mentioned previously it is known to apply lacquers and varnishes f. i. copal lacquers to waxed meerschaum pipes.

35 In contradiction to the known methods the invention is based on the new discovery that the waxing treatment may be entirely eliminated if diluted solutions of synthetic resins are adopted for the treatment of the shaped article; in other words the known treating methods for meerschaum pipes which embrace a plurality of different operating stages namely waxing, oiling and lacquering or varnishing are replaced in the present case by the sole treatment with solutions of synthetic resins.

40 45 This treatment may be improved by using a solution of a plurality or a mixture of different synthetic resins, which are selected in order to vary the lustre and color or the mechanical properties of the treated articles.

50 In conformity with the objects of this invention the pipes are impregnated or treated therefore with a uniform substance only and the source of blister creation is eliminated.

The lustre and the color of the finished product and its resistance to impacts and to breakage

equals that of a pipe which is cut from the best quality meerschaum.

Furthermore it is possible to conceal folds, fissures, cracks resulting from the manufacturing process by applying to the article a coating of colored or white synthetic resin solutions, whereas in similar cases with waxed pipes ornamental designs are applied to the faulty surface which considerably lessens the commercial value of the article.

In accordance with my invention the shaped meerschaum pipes are coated or impregnated and coated with a diluted solution of a synthetic resin in a suitable organic solvent.

Though my novel process may be performed in any desired manner I prefer to treat the pipes, as follows:

The shaped article is impregnated with or immersed in a diluted solution of a synthetic resin e. g. of the urea or phenol-formaldehyde type. Known organic solvents e. g. butyl alcohol and xylol may be used to prepare the solution. The concentration of the diluted solution may vary between about 5 to 35%, however the more diluted solutions are preferable. The synthetic resin solution may also be added into the mold where the meerschaum pipe is subjected to the moulding action. The treatment with the synthetic resin solution may last several hours. Thereupon the article is dried at a temperature of approximately between 150 to 350° F. After this a coating of the same or of another synthetic resin solution may be applied to the article which then is dried again.

#### Example

A pipe moulded of meerschaum powder in the usual manner is heated for approximately one hour at approximately 300° F. in order to remove the last traces of moisture. The pipe is thereupon immersed for approximately eight hours in a 20% xylol solution of a synthetic urea resin which solution is heated to approximately 170° F. The pipe is then dried for four hours. The

whole procedure may be repeated. Thereupon a coating of a white or colored synthetic resin liquor is applied and the pipe is then dried for approximately 30 minutes at about 300° F.

I claim:

1. Process for the manufacture of meerschaum pipes from pulverulent meerschaum consisting in molding the pipe from said powder impregnating the molded pipe with a diluted and heated solution of at least one substance selected from the group consisting of phenol formaldehyde and urea resins, drying the article, applying to the same a coating of the same type resins and hardening said coating.

10 2. Process for the manufacture of meerschaum pipes from pulverulent meerschaum consisting in molding the pipe from said material, heating the same to entirely remove the moisture, dipping the pipe for approximately eight hours in a solution containing 5 to 35% of at least one substance selected from the group consisting of phenol formaldehyde and urea resins, drying the same at a temperature of approximately 170° F., applying to the same a coating of the same type resins and hardening the same at a temperature of approximately 300° F.

20 3. Process for the manufacture of meerschaum pipes from pulverulent meerschaum consisting in molding the pipe from said powder impregnating the molded pipe with a diluted solution of at least one substance selected from the group consisting of phenol formaldehyde and urea resins, drying the article, applying to the same a coating of the same type resins and hardening said coating.

30 4. Process for the manufacture of meerschaum pipes from pulverulent meerschaum consisting in molding the pipe from said powder, impregnating and coating the molded pipe with a solution of at least one substance selected from the group consisting of phenol formaldehyde and urea resins, drying the article and hardening the said coating.

ERNEST LICHTBLAU.